

May 4, 1937.

J. A. MITCHELL

2,079,379

COATED MATERIAL AND METHOD OF MAKING SAME

Filed May 3, 1934

2 Sheets-Sheet 1

FIG. 1.



FIG. 2.



INVENTOR.

James A. Mitchell  
BY

Charles F. Daley  
ATTORNEY.

May 4, 1937.

J. A. MITCHELL

2,079,379

COATED MATERIAL AND METHOD OF MAKING SAME

Filed May 3, 1934

2 Sheets-Sheet 2

FIG. 3



FIG. 4



INVENTOR.  
BY James A. Mitchell

Charles F. Daly  
ATTORNEY.

## UNITED STATES PATENT OFFICE

2,079,379

COATED MATERIAL AND METHOD OF  
MAKING SAME

James A. Mitchell, Kenmore, N. Y., assignor, by  
mesne assignments, to E. I. du Pont de Nemours  
& Company, Wilmington, Del., a corporation of  
Delaware

Application May 3, 1934, Serial No. 723,787

8 Claims. (Cl. 91—68)

This invention relates to moistureproofing compositions and to means for producing them. It relates more particularly to moistureproof sheet materials having improved surface characteristics 5 both as regards their ability to maintain their individuality under normal conditions of storage and their ability to be mutually sealable upon the application of heat.

With the modern trends of development in the packaging of commodities, especially perishable foodstuffs, the need has arisen for a wrapping material which can at once provide physical protection against contamination, preservative action by retaining within the package the original conditions such as moisture content, and sales appeal by permitting examination of the package contents without destroying the wrapper. These needs have been largely fulfilled by the recent introduction to the trade of a wrapping material comprising a transparent base sheet, such as regenerated cellulose, coated with a transparent moistureproofing composition, which latter may comprise a cellulose derivative, a wax, a resin or blending agent and a plasticizer.

Prior art wrapping materials were generally of the character of waxed papers and could be at least superficially joined by means of heat and pressure. The wrapping industry is generally provided with expensive equipment designed for heat sealing and will look with favor on new materials only if they can be adapted to this equipment. Moistureproof wrapping materials such as the coated regenerated cellulose described above also have the property of being heat sealable to a degree, but the joint is not sufficiently rugged to satisfy the current demands.

These moistureproof wrapping materials are furnished to the consumer in the form of continuous roll stock or as cut-to-size sheets. In order that the roll stock will unroll smoothly or the cut-to-size sheets separate easily, the surface of the material must be smooth and non-tacky and there must be no tendency towards caking or sticking together during the time of storage which intervenes between manufacture and consumption. The moistureproofing composition, on the other hand, must be flexible, transparent and sufficiently thermoplastic to permit intermingling of superposed coatings during the brief period of the heat sealing operation with immediate set-up thereafter although it cannot be so thermoplastic that it will be affected by the temperature variations normally encountered in handling or storage.

One object of this invention comprises the pro-

duction of improved moistureproof film. A further object of the invention relates to improvements in the manufacture of heat-sealable moistureproof wrapping tissues. A further object of the invention relates to the production of moistureproof wrapping tissues which fulfill the requirements for flexibility and transparency and additionally possess a high degree of surface smoothness, slip and resistance to sticking under storage conditions. Further objects of the invention will appear hereinafter.

This invention is primarily concerned with moistureproofing compositions comprising a cellulose nitrate, a moistureproofing agent, a plasticizer and a resin or other blending agent. The term "moistureproofing agent" defines the material which serves as the basis for moistureproofness. In the formulation of cellulose nitrate coating compositions it is well known in the art to use a plasticizing agent to impart flexibility to the coating. This is also true in the formulation of cellulose nitrate coating compositions which contain moistureproofing agents, but it has been observed that the plasticizer also contributes to the moistureproofing property and for the production of highly moistureproof coating compositions more plasticizer is employed than is necessary merely for its plasticizing action. The use of excess plasticizer to accomplish this purpose, however, tends to impair the surface characteristics of the moistureproofing coating composition since with increased plasticizer content the composition becomes softer, stickier and more thermoplastic. The softness and stickiness are objectionable from the point of view of good surface slip and storage. The increased thermoplasticity would be advantageous for the improvement of heat sealing properties were it not for the fact that the minimum amount of plasticizer which will afford good heat sealing is so close to the amount which will still avoid softness and tackiness that the practical control of such a composition to insure a coated product of uniformly good heat sealing properties and uniformly good surface characteristics is extremely difficult, especially for the commercial production of a continuous coated sheet material. Indeed, many common plasticizers pass the point which is critical for good surface before the point of satisfactory heat seal is reached.

For the purposes of this invention, moistureproof materials are defined as those which, in the form of a thin, continuous and unbroken sheet or film, will permit the passage of not more than 690 grams of water vapor per 100 square meters per

hour over a period of 24 hours at approximately 39.5° C. plus or minus 0.5° C., the relative humidity of the atmosphere at one side of the film being maintained at least at 98% and the relative humidity of the atmosphere at the other side being maintained at such value as to give a humidity differential of at least 95%.

Moistureproofing coating compositions are defined as those which, when laid down in the form of thin, continuous, unbroken films, applied uniformly as a coating with a total coating thickness not exceeding 0.0005" to both sides of a sheet of regenerated cellulose of thickness approximately 0.0009", will produce a coated product which is moistureproof.

For the purposes of experimental tests, especially for those materials adaptable as coating compositions, moisture proof materials include those substances, compounds or compositions which, when laid down in the form of a continuous, unbroken film applied uniformly as a coating with a total coating thickness not exceeding 0.0005" to both sides of a sheet of regenerated cellulose of thickness approximately 0.0009" will produce a coated sheet which will permit the passage therethrough of not more than 690 grams of water vapor per 100 square meters per hour over a period of approximately 24 hours, at a temperature of 39.5° C. plus or minus 0.5° C. (preferably 39.5° C. plus or minus 2.5° C.) with a water vapor differential of 50-55 mm. (preferably 53.4 plus or minus 0.7 mm.) of mercury. For convenience the number of grams of water vapor passed under these conditions may be referred to as "permeability value". An uncoated sheet of regenerated cellulose having a thickness of approximately 0.0009" will show a permeability value of the order of 6900.

In the foregoing, it is apparent that under the conditions set forth, a moistureproofed regenerated cellulose sheet is capable of resisting the passage of moisture or water vapor therethrough at least ten times as effectively as the uncoated regenerated cellulose sheet.

The composition may be coated on to the base to give a wide range of coating thicknesses, and where heat sealing is desired, increase in the coating thickness will increase the heat sealing property of any given composition. For the purpose of this invention, and particularly where the ultimate coated sheet material is to be used as a wrapping tissue, the coating thickness is 0.00002" to 0.0005" and preferably 0.00005" on each side of the base.

When heat sealing properties are desired, it will be found that sheet materials provided with compositions described in this specification are truly heat sealable in the sense that a heat sealed joint will be stronger than a joint sealed by means of acetone. Additionally, the joint will be at least as strong as a solvent sealed joint obtained by means of methoxy ethanol. These same considerations apply to films obtained by casting the coating compositions per se.

As indicative of the strength of the heat sealed joint obtainable, the following test has been devised:

Strips of the coated material 1.5" wide are superposed on one end so that opposite faces of the film are in contact. A seal is made across the width of the material by imposing thereon a heated iron weighing 1500 grams for 2 seconds. The iron is so designed as to cause a seal to be made of a width of 2/32", the iron being maintained in any suitable manner at a temperature

above 130° C. and below 200° C. as, for instance, 150° C. The two strips so sealed are opened at the free ends and placed in a stretching device, such as a Suter testing machine, by gripping each end of the sheet in suitable clamps, one of which is fixed while the other is moved away at a constant speed of 12" per minute. The force in grams required to pull the sheets apart is taken as a measure of the bond strength and may be referred to as "heat sealing value".

In accordance with this invention, it has now been found that there are certain plasticizers for cellulose nitrate-moistureproofing agent coating compositions which are unique in their ability to plasticize, increase moistureproofness, provide excellent surface and storage characteristics and also impart a high degree of thermo-plasticity which can in turn produce an exceptionally strong heat sealed joint. Dicyclohexyl phthalate and cyclohexyl acid phthalate are the plasticizers which possess this unique property. They may be used alone or in combination with other common plasticizers to produce moistureproofing coatings which exhibit a high degree of moistureproofness; good appearance, flexibility and transparency; excellent surface slip and storage without sticking or marring; and excellent heat sealing properties. Among the plasticizers which may be advantageously combined with dicyclohexyl phthalate or cyclohexyl acid phthalate are alkyl phthalates such as dibutyl phthalate, tricresyl phosphate, dicyclohexyl adipate, esters of o-benzoyl benzoic acid, cyclohexyl butyl phthalate, derivatives of toluene sulfonamide and the like. Throughout the balance of this specification reference will be made to dicyclohexyl phthalate, but it is to be understood that cyclohexyl acid phthalate may be advantageously employed although because of its somewhat superior properties, the former is to be preferred.

I have found that cellulose nitrate coating compositions plasticized with dicyclohexyl phthalate exhibit unique properties which may account for the improved surface and storage characteristics. Thus, for example, a composition of nitrocellulose, resin and dicyclohexyl phthalate exhibits no plasticity at ordinary temperatures; at least, a film cast from such a composition undergoes no deformation under tensile stress and has a high breaking strength. On the other hand, the composition is thermoplastic and becomes heat-sealable at elevated temperatures. It is apparent, then, that when a sheet of base material such as regenerated cellulose is coated with a composition of this type the coating retains its normal characteristics. Consequently, the coated sheets will possess good surface slip, and will not be subject to caking, sticking or marring in storage because the coating suffers no deformation under the stresses encountered in storage. The thermoplasticity of the coating at elevated temperatures, however, affords excellent heat-sealing properties. The same considerations are applicable to compositions comprising a moisture-proofing agent.

Generally speaking, the coating compositions embodied in this invention comprise dicyclohexyl phthalate or cyclohexyl acid phthalate in combination with a cellulose nitrate, a moisture-proofing agent and preferably a resin or blending agent. In addition, other plasticizers, drying or non-drying oils, additional resinous material of either the natural or synthetic varieties, coloring agents either as dyes or pigments, or other modifying agents may be used accord-

ing to the type of coating composition desired. Obviously, for those uses where a transparent coated material is desired, any pigments or modifying agents which will impair the transparency of the coating composition will be omitted therefrom. The proportions of the several ingredients may vary within rather wide limits, depending on the properties desired in the finished composition and these will be more specifically set forth below and will be illustrated in the several examples.

The invention contemplates only those coating compositions which comprise a cellulose nitrate. Cellulose nitrates of varying degrees of conversion such as of various nitrogen contents may be used and, indeed mixtures of different types of cellulose nitrate may also be used as, for example, mixtures of cellulose nitrates of different nitrogen contents. Cellulose nitrate of low nitrogen content such as 11.5% nitrogen, is generally preferable especially where high heat sealability is desired.

As additional plasticizers for use in combination with those of this invention, it is possible to use any of the plasticizers mentioned previously as well as such compounds as dilauryl phthalate, di-(methylcyclohexyl) phthalate, di-(dimethylcyclohexyl) phthalate, methyl-(dimethylcyclohexyl) adipate, or the like.

As moistureproofing agents, it is possible to use waxes or wax-like materials such as paraf-

compatibility of these two ingredients. This material is referred to as a blending agent and is usually of a resinous nature although this is not absolutely necessary. When the blending agent is resinous, advantage may be taken of its film-forming characteristics, if any, and sufficient quantity may be added to a coating composition to contribute towards the body and build of that composition in addition to the blending action. Depending on the nature of the blending agent, more or less plasticizing action on the cellulose nitrate may be obtained.

As blending agents, any of the natural or synthetic resins commonly available may be used so long as they are compatible and form homogeneous mixtures. Such resins may include ester gum, rosinates, hydrogenated rosin, hydrogenated rosin esters, damar, copal, kauri, glyptals, vinyl derivatives, chlorinated diphenyl resins, soluble resins of the phenol-formaldehyde type. Non-resinous blending agents may be used when they yield homogeneous mixtures and these may include hydrogenated castor oil, castor oil phthalate, lanolin or wool grease, ethyl abietate, methyl abietate, diethylene glycol rosinate, diethylene glycol hydrorosinate or the like.

As illustrative of moistureproofing coating compositions which embody the principles of this invention, the following specific examples are given but they should not be considered in any way as limitative of the scope of this invention.

Table I

| 35                          | Solids composition by weight    | Examples |      |      |      |      |      |      |      |      |      |     | 35 |
|-----------------------------|---------------------------------|----------|------|------|------|------|------|------|------|------|------|-----|----|
|                             |                                 | I        | II   | III  | IV   | V    | VI   | VII  | VIII | IX   | X    | XI  |    |
| <i>Cellulose derivative</i> |                                 |          |      |      |      |      |      |      |      |      |      |     |    |
| 40                          | Nitrocellulose (11.5% N)        | 48.0     | 57.5 | 47.9 | 49.9 | 49.0 | 50.0 | 11.7 | 54.0 | 51.0 | 40   |     |    |
|                             | Nitrocellulose (12.5% N)        |          |      |      |      | 50.1 | 64.0 | 38.5 |      |      |      |     |    |
| <i>Plasticizer</i>          |                                 |          |      |      |      |      |      |      |      |      |      |     |    |
| 45                          | Dicyclohexyl phthalate          | 43.0     | 18.1 | 32.0 | 30.0 | 16.5 | 32.0 | 30.0 | 21.8 | 21.0 | 22.0 |     |    |
|                             | Cyclohexyl acid phthalate       |          |      |      |      | 33.9 |      |      |      |      |      |     |    |
|                             | Dibutyl phthalate               | 6.0      |      | 10.0 | 16.5 |      |      | 7.3  | 7.0  | 10.0 | 45   |     |    |
|                             | Dilauryl phthalate              |          |      | 10.0 |      |      |      |      |      |      |      |     |    |
| <i>Blending agent</i>       |                                 |          |      |      |      |      |      |      |      |      |      |     |    |
| 50                          | Dewaxed damar                   | 6.7      |      | 7.5  | 7.5  | 14.0 | 12.0 |      | 16.7 |      | 13.0 |     |    |
|                             | Ester gum                       |          |      |      |      |      |      |      |      |      |      |     |    |
|                             | Methyl abietate                 | 14.4     |      |      |      |      |      |      |      |      |      |     | 50 |
|                             | Ethyl abietate                  |          |      |      |      |      |      |      |      |      |      |     |    |
|                             | Diethylene glycol rosinate      |          |      |      |      |      |      | 13.0 |      | 14.0 |      |     |    |
|                             | Diethylene glycol hydrorosinate |          |      |      |      |      | 14.0 |      |      |      |      |     |    |
| <i>Wax</i>                  |                                 |          |      |      |      |      |      |      |      |      |      |     |    |
| 55                          | Asiatic paraffin                | 2.3      | 4.0  | 2.6  | 2.6  | 4.0  | 4.0  | 4.0  | 3.0  | 4.0  | 4.0  | 4.0 | 55 |

fin, petrolatum, ceresin, Japan wax, palm wax, beeswax, certain chlorinated hydrocarbons, Chinese insect wax or other synthetic waxes or wax-like material. If some of these waxes are too soft for the purposes desired, they may be mixed with harder waxes of the group or with carnauba wax, candelilla wax or other harder waxes. Generally, paraffin serves as a satisfactory moistureproofing agent which may be hardened if necessary by admixture with carnauba or candelilla wax. In the examples which accompany this specification, Asiatic paraffin has been employed as typical of a highly satisfactory moistureproofing agent, but it is to be understood that other moistureproofing agents may be substituted.

In the preparation of moistureproofing coating compositions comprising a cellulose nitrate and a moistureproofing agent, it is advantageous to include some material which will improve the

When the heat seal test described above is applied to sheets of regenerated cellulose coated with a moisture-proofing coating composition such as that of Example IV so that the total coating thickness is approximately 0.0001" (approximately 3 grams of composition solids per square meter for both sides), a heat sealing value of the order of 180 is obtained. Other examples which are typical of good heat sealable compositions may be chosen within the range 60 represented as satisfactory by means of the accompanying curves III and IV of Fig. 3 and comparable heat sealing values will be obtained. These heat sealing values are to be considered as merely illustrative of the bond strength attainable since it is obvious that greater or lesser bond strengths may have many useful applications, depending on the use to which the coated base material is put.

It is most convenient to apply the above mois-

tureproofing coating compositions to base materials such as sheets of regenerated cellulose by means of suitable solvents. Thus, the film-forming ingredients, conveniently considered as solids, indicated in any of the above examples may be dissolved to give a coating solution of appropriate viscosity and solids content whereupon the solution may be applied to the desired base in accordance with the methods known to the art. The solvents may be removed and the coated base subjected to an elevated temperature at least equal to the melting point of the wax, whence, after cooling, a clear, transparent, moisture-proof coated base will be obtained. A suitable technique for this operation is set forth in Charch and Prindle U. S. Patent No. 1,737,187 and since it is not a part of this invention, no further discussion seems necessary.

For the specific examples set forth, the following solvent mixtures may be successfully employed:

Table II

| Solvent            | Examples using pyroxylin containing |                          |                                   |                          |
|--------------------|-------------------------------------|--------------------------|-----------------------------------|--------------------------|
|                    | 11.5% N                             |                          | 12.5% N                           |                          |
|                    | Range                               | Preferred                | Range                             | Preferred                |
| Ethyl alcohol..... | Percent<br>4-18<br>24-50<br>45-70   | Percent<br>8<br>33<br>59 | Percent<br>0-10<br>25-50<br>45-70 | Percent<br>2<br>37<br>63 |
| Toluene.....       |                                     |                          |                                   |                          |
| Ethyl acetate..... |                                     |                          |                                   |                          |

These solvent mixtures may be modified by the addition of other well known lacquer solvents to obtain special drying effects without in any way affecting the unique properties of dicyclohexyl phthalate or cyclohexyl acid phthalate as set forth in this specification.

These moistureproofing compositions may be applied to various sheet materials to produce wrapping tissues which are flexible, moistureproof and heat sealable and which exhibit highly improved surface characteristics including excellent surface slip and resistance to caking, sticking or marring during storage. A variety of base sheet materials may be used such as cellulosic materials, paper, albuminous materials (gelatin, agar-agar, casein), or films made from rubber derivatives, e. g., the material prepared by reacting rubber and a metal halide such as boron trifluoride, stannous or stannic chloride, stannic acid, and other materials which are disclosed in an article by Thies and Clifford in the "Journal of Industrial and Engineering Chemistry", vol. 26, page 123 (1934), the method of reacting the materials conforming to that disclosed in the said article referred to. In the preferred embodiment of the invention, a non-porous, non-fibrous, dense, smooth surfaced and preferably transparent material, such as regenerated cellulose, cellulose ester films including cellulose nitrate and cellulose acetate, or cellulose ether films including ethyl cellulose, benzyl cellulose, glycol cellulose or lowly etherified cellulose, such as those in which there is only one substituent group for several glucose units of cellulose, is employed. It is obvious that suitable solvent adjustment will be made in the formulation of moistureproofing coating compositions of the type described in order that there may be no harmful effect on the base material employed.

In the coating compositions set forth in the above examples it is apparent that the propor-

tions of the several ingredients may be varied over a considerable range. Thus, the cellulose nitrate may comprise 40-65% or more of the total solids although in most instances 45-55% will be found most satisfactory with approximately 50% a convenient, generally useful proportion. The ratio of cellulose nitrate to blending agent may vary over a wide range from 2:1 to 8:1, or even greater, but, for most purposes, a ratio from 3:1 to 7:1 is satisfactory while a ratio of 4:1 is convenient and yields generally good results. The cellulose nitrate is usually in excess of the total plasticizer content and the ratio of cellulose nitrate to plasticizer may vary from 1:1 to 3:1, but a ratio of 1.5:1 to 2:1 is generally found to give the best results.

The blending agent may vary according to the cellulose nitrate, plasticizer or moistureproofing agent employed and it may constitute 1-20% or more of the total solids. When highly heat sealable compositions are desired, the amount of blending agent is preferably low and may comprise 5-10% or less of the total solids. The ratio of blending agent to moistureproofing agent may vary from 1:5 or less to 5:1 or more, and usually a ratio of approximately 3:1 to 4:1 will be found satisfactory. The larger amounts of blending agent are usually used when the blending agent exerts some plasticizing action and can therefore replace a portion of the plasticizer.

The moistureproofing agent is usually present in a quantity sufficient to impart a suitable degree of moistureproofness while still maintaining homogeneity of composition so that the ultimate moistureproofing coating on the moistureproof article prepared in accordance with the invention will be clear, transparent, non-greasy, non-smearable and non-tacky under the normal conditions of handling or storage. Generally speaking, if the moistureproofing agent constitutes less than 10% of the total solids, these conditions will be fulfilled but while 2-6% of moistureproofing agent has been found to yield excellent results, it is to be understood that more or less may be used, depending on the nature of the moistureproofing agent.

The plasticizer must be either dicyclohexyl phthalate or cyclohexyl acid phthalate or a mixture of plasticizers containing appreciable quantities of one or both of these specific compounds if the objects of the invention are to be accomplished. The total plasticizer concentration may vary from 20-45% of the total solids. Low percentages of plasticizer, however, are usually used only when the blending agent is capable of exerting a plasticizing action and can therefore substitute for a portion of plasticizer which might otherwise be added. Among the objects of this invention is the production of highly moistureproof and preferably highly heat sealable coating compositions and for the accomplishment of this object it is usually necessary to use relatively large amounts of plasticizer and as illustrated in the accompanying examples, the use of 30-40% or more of plasticizer is preferable. When the total plasticizer comprises substances other than dicyclohexyl phthalate or cyclohexyl acid phthalate, such, for example, as dibutyl phthalate or a plasticizing blending agent, it is preferable that the dicyclohexyl phthalate or cyclohexyl acid phthalate predominate. Usually, 50% or more of the total plasticizer should be provided by these substances although as little as 25% or even less may be used with certain plasticizers without completely eliminating the unique properties

of these specific plasticizers. Because of the desired high percentage of plasticizer in the total composition the ratio of plasticizer to moisture-proofing agent may be quite high, in some instances amounting to as much as 20:1. On the other hand, if a plasticizing-blending agent is used, the ratio of plasticizer to moistureproofing agent may fall as low as 6:1. Usually, a ratio of 7:1 to 10:1 will be found to serve satisfactorily.

10 In the preceding discussion of the proportions of ingredients in the coating compositions the ranges of percentage composition or ratio have been given to facilitate the formulation of highly satisfactory and preferred compositions, and to aid one skilled in the art in quickly and easily arriving at operable compositions not specifically described in the examples. It is to be understood, however, that these limiting ranges are largely illustrative and do not restrict the invention beyond the limitations set forth in the appended claims.

Numerous advantages of the invention may be observed by reference to the accompanying drawings.

25 Referring to Fig. 1, a series of curves will be observed which represent the change in permeability value for a given moistureproofing composition with increasing plasticizer concentration. The curves were all obtained by substituting different plasticizers in the same basic composition in which latter the moistureproofing agent constituted 4% of the total solids while the ratio of cellulose nitrate to blending agent remained constant at 4:1. Nitrocellulose containing 11.5% 30 nitrogen was used. Curve I represents the results obtained using dibutyl phthalate as the plasticizer while curve II was obtained by the use of tricresyl phosphate and curve III by the use of either dicyclohexyl phthalate or cyclohexyl acid phthalate. The broken line portions of the curves indicate compositions which have poor surface characteristics including poor slip and tendency to cake, stick or smear during storage. It is apparent that increase in plasticizer content increases moistureproofness, as is evidenced by the marked decrease in permeability value. It will be noted however that in the range of high moistureproofness (permeability values of 40 or less), both Curves I and II show that increase of 45 plasticizer concentration is detrimental to the surface characteristics of the coating compositions. Thus, the use of more than 29% dibutyl phthalate or 32% of tricresyl phosphate results in the production of a soft and sticky coating 50 composition. On the other hand, curve III shows that the specific plasticizers of this invention continue to improve the moistureproofness without any harmful effects on the surface characteristics.

55 Fig. 2 illustrates the same points as Fig. 1, using a nitrocellulose having a nitrogen content of 12.5%. Here again, the curve III definitely indicates the superiority of dicyclohexyl phthalate or cyclohexyl acid phthalate as plasticizers for highly moistureproof coating compositions having extraordinary surface characteristics.

Fig. 3 provides a series of curves obtained from a study of coating compositions formulated to secure good heat sealing properties in addition to moistureproofness and good surface characteristics. All of these compositions contained 3% Asiatic paraffin as the moistureproofing agent, 7% damar (dewaxed) as the blending agent and sufficient pyroxylin of 11.5% nitrogen 70 content. The broken portions of the curves re-

present compositions having unsatisfactory heat sealing power as defined above. It is apparent that satisfactory heat sealing cannot be obtained with dibutyl phthalate or tricresyl phosphate (curves I and II) until the plasticizer content is 5 in excess of approximately 35%. Dicyclohexyl phthalate alone (curve IV) is satisfactory over 38% and the mixed plasticizer of curve III becomes effective at about the same concentration.

The curves represented in Fig. 4 are identical 10 with those of Fig. 3 but the broken portions indicate compositions which show unsatisfactory surface characteristics.

A comparison of the curves in Figs. 3 and 4 reveals that in the curves I and II compositions 15 having satisfactory heat sealing properties have unsatisfactory surface characteristics. As a matter of fact, in both curves the critical point for good surface is passed before a satisfactory 20 heat seal is reached. On the other hand, compositions plasticized wholly or in part by dicyclohexyl phthalate (curves III and IV) show 25 good surface characteristics throughout the entire range.

From the foregoing, it is apparent that moistureproofing coating compositions comprising a cellulose nitrate, a moistureproofing agent and a blending agent, and plasticized wholly or in part by means of dicyclohexyl phthalate or cyclohexyl acid phthalate possess numerous advantages over the prior art, making possible the production of moistureproof sheet materials suitable for use as wrapping tissues which have superior qualities. Sheet materials coated with these 30 compositions have excellent surface slip and are highly resistant to caking, sticking or smearing under conditions normal to storage. When the base sheet material is transparent, the final product is also transparent unless the coating 35 compositions are deliberately modified to produce opaque, colored or otherwise preferred effects. The compositions, and hence the coated sheet materials, can be made moistureproof over a comparatively wide range of permeability values and where a high degree of moistureproofness is desired, this too can be obtained without deleteriously affecting the surface characteristics of the product. At the same time a highly 40 heat sealable wrapping tissue with high moistureproofness and good surface characteristics 45 may be obtained. The unique effect of these specific plasticizing agents is highly unobvious and their use provides new and useful moistureproofing coating compositions and coated sheet materials, thus constituting a marked advance 50 in the art.

Where percentages and proportions are referred to throughout the specification, they represent parts by weight unless indicated otherwise.

Any modification or variation of the invention as described above, which conforms to the spirit of the invention, is intended to be included within the scope of the claims.

I claim:

1. A heat sealable, moistureproof, non-porous, non-fibrous, wrapping tissue having good surface slip and good storage characteristics, comprising a non-porous, non-fibrous base and a coating thereon containing pyroxylin containing 10.5 to 70 11.5% nitrogen, a wax material, a blending agent and a plasticizer comprising dicyclohexyl phthalate, the pyroxylin comprising about 40-65% of the total solids in the coating, the pyroxylin-blending agent ratio being from 2:1 to 8:1, the 75

- pyroxylin-plasticizer ratio being about 1:1 to 3:1, and the blending agent wax material ratio being about 1:5 to 5:1.
2. A heat sealable, moistureproof, non-porous, 5 non-fibrous, wrapping tissue having good surface slip and good storage characteristics, comprising a non-porous, non-fibrous base and a coating thereon containing pyroxylin containing 10.5 to 11.5% nitrogen, a wax material, a blending agent and a plasticizer comprising dicyclohexyl phthalate, the pyroxylin comprising about 45-55% of the total solids in the coating, the pyroxylin-blending agent ratio being about 4:1, the pyroxylin-plasticizer ratio being about 1.5:1 10 to 2:1, the blending agent wax material ratio being about 3:1 to 4:1, being further characterized in that the plasticizer is predominantly a cyclohexyl phthalate.
3. A moistureproofing coating composition 20 which is heat-sealable when dry comprising pyroxylin containing 10.5 to 11.5% nitrogen, a wax material, a resin and a plasticizer comprising dicyclohexyl phthalate, the pyroxylin comprising about 40-65% of the total solids, the pyroxylin-blending agent ratio being from 2:1 to 8:1, the 25 pyroxylin-plasticizer ratio being about 1:1 to 3:1, and the blending agent wax material ratio being about 1:5 to 5:1.
4. A moistureproofing coating composition 30 which is heat-sealable when dry comprising pyroxylin containing 10.5 to 11.5% nitrogen, a wax material, a resin and a plasticizer comprising dicyclohexyl phthalate, the pyroxylin comprising about 45-55% of the total solids, the pyroxylin-blending agent ratio being about 4:1, the pyroxylin-plasticizer ratio being about 1.5:1 to 2:1 35 the blending agent wax material ratio being about 3:1 to 4:1, being further characterized in that the plasticizer is predominantly a cyclohexyl phthalate.
5. A transparent heat sealable, moistureproof, non-fibrous, substantially non-porous pellicle, having good surface slip and good storage char-

acteristics, comprising a non-porous, non-fibrous base and a moistureproofing coating thereon containing a wax material, pyroxylin, and a plasticizer taken from the group consisting of dicyclohexyl phthalate and cyclohexyl phthalate, the pyroxylin comprising 40 to 65% of the total solids of the coating, and the pyroxylin-plasticizer ratio ranging from about 1:1 to 3:1. 5

6. A transparent, heat sealable, moistureproof, non-fibrous, substantially non-porous pellicle having good surface slip and good storage characteristics, comprising a regenerated cellulose base and a moistureproofing coating thereon containing a wax material, pyroxylin, and a plasticizer composed of a mixture of a liquid 15 plasticizer and a solid plasticizer, the solid plasticizer taken from the group consisting of dicyclohexyl phthalate and cyclohexyl acid phthalate, in which the solid plasticizer predominates, the pyroxylin comprising 40 to 65% of the 20 total solids of the coating, and the pyroxylin-plasticizer ratio ranging from about 1:1 to 3:1.

7. A moistureproofing coating composition 25 which is heat sealable when dry comprising pyroxylin, a wax material, and a plasticizer taken from the group consisting of dicyclohexyl phthalate and cyclohexyl acid phthalate, the pyroxylin comprising 40 to 65% of the total solids of the coating, and the pyroxylin-plasticizer ratio ranging from about 1:1 to 3:1. 30

8. A moistureproofing coating composition which is heat sealable when dry comprising pyroxylin, a wax material, and a plasticizer composed of a mixture of a liquid plasticizer and a solid plasticizer, the solid plasticizer taken from the group consisting of dicyclohexyl phthalate and cyclohexyl acid phthalate, in which the solid plasticizer predominates, the pyroxylin comprising 40 to 65% of the total solids of the coating, and the pyroxylin-plasticizer ratio ranging from 40 about 1:1 to 3:1. 35

JAMES A. MITCHELL.